

April 3, 1951

P. F. GEORGE ET AL

2,547,909

PRIMARY CELL

Filed May 7, 1949

2 Sheets-Sheet 1



Fig. 4



Fig. 1

INVENTORS.

Percy F. George  
Ashford B. Fry  
Roy C. Kirk

BY *Griewold & Burdick*  
ATTORNEYS

April 3, 1951

P. F. GEORGE ET AL  
PRIMARY CELL

2,547,909

Filed May 7, 1949

2 Sheets-Sheet 2



Mg alloyed with 0.16 to 0.7% of Hg, Fe <0.007%



Mg alloyed with 0.16 to 0.7% of Hg, Fe <0.007%

INVENTORS.  
Percy F. George  
Ashford B. Fry  
Roy C. Kirk  
BY Griswold & Gurdick  
ATTORNEYS

## UNITED STATES PATENT OFFICE

2,547,909

## PRIMARY CELL

Percy F. George, Ashford B. Fry, and Roy C. Kirk,  
Midland, Mich., assignors to The Dow Chemical  
Company, Midland, Mich., a corporation of  
Delaware

Application May 7, 1949, Serial No. 91,928

2 Claims. (Cl. 136—100)

1

The invention relates to primary cell anodes. It more particularly concerns an improved primary cell anode employing an aqueous electrolyte and magnesium in the anode material.

Inasmuch as magnesium is an abundant and readily available metal high in the electromotive force series of metals numerous attempts have been made heretofore to utilize the metal as the anode material in primary cells, especially those employing an aqueous electrolyte. However, the anodes in such cells have not generally exhibited a satisfactory electrochemical efficiency. That is to say the actual number of coulombs of electricity produced per gram of the anode material consumed falls far short of 7940, the theoretical number of coulombs per gram of magnesium.

It is the principal object of the invention to provide an improved primary cell anode employing magnesium as the anode material with enhanced efficiency. Other objects and advantages will appear as the description of the invention proceeds.

The invention is predicated upon the discovery that by alloying a small amount of mercury i. e. between about 0.16 and 0.7 per cent by weight with the magnesium and limiting the iron content of the resulting alloy to less than about 0.007 per cent, as by using purified magnesium, a greatly enhanced electrochemical efficiency is obtained on using the alloy as anode material in a primary cell having an aqueous electrolyte. The invention then consists of the improved primary cell anode hereinafter fully described and particularly pointed out in the claims.

In carrying out the invention, magnesium containing up to about 0.007 per cent of iron is used. The usual commercial grades of magnesium generally contain more iron than can be tolerated in the anode material of this invention, and if used, should first be purified as by distillation. In alloying the mercury, the conventional melting and alloying practices of the magnesium foundry may be used. The mercury may be added as by pouring the requisite amount into the molten magnesium which may be protected from atmospheric attack by the usual saline flux. The melt preferably is stirred after the addition of the mercury to insure uniformity of distribution of the mercury throughout the magnesium. In general the mercury content may be between 0.16 and 0.7 per cent as aforesaid, however best results appear to be obtained when the mercury content is about 0.5 per cent and the iron content not over about 0.002 per cent. After alloying, the melt may be cast and worked into any

5 desired shape of anode by any of the conventional fabrication procedures known in the art of working magnesium alloys, such as extrusion, rolling, and forging and combinations of these operations.

Primary cells of either the "wet" or "dry" type may be constructed employing the anode material of the invention in combination with any suitable cathode and in aqueous electrolyte. As electrolytes any of the various aqueous electrolytes that have been suggested heretofore for voltaic systems employing a magnesium or magnesium base alloy anode may be used with the anode of the invention. The preferred electrolyte is that disclosed in our patent application Serial No. 73,063 filed January 27, 1949, when the electrolyte is used in combination with a manganese dioxide depolarized cathode.

10 The aqueous electrolyte of the said patent application comprises a bromide of an alkali or alkaline earth metal, the electrolyte advantageously containing corrosion inhibiting amounts of a chromic acid salt of a base consisting of an alkali metal base or an alkaline earth metal base including magnesium and ammonium. Of the various bromides above indicated which may be used in solution in water as the electrolyte, magnesium bromide either alone or in combination with lithium bromide is to be preferred. Suitable concentrations are from about 150 to 500 grams per liter, the upper limit of concentration being the solubility of the bromide in water. A generally suitable concentration is about 300 grams per liter. While various electronic conductors that are not attacked by the electrolyte may be used for the cathode such as carbon, graphite, platinum, we prefer to use carbon. The invention may be further explained by reference to the accompanying drawing in which:

15 Fig. 1 is a graph showing the relationship between the efficiency of the anode material in per cent and the percentage of mercury in the anode, the iron content of the anode being about 0.002 per cent.

20 Fig. 2 is an end elevation of a "wet" test cell embodying the anode of the invention.

25 Fig. 3 is a front elevation of the anode of the cell of Fig. 2.

30 Fig. 4 is a preferred form "wet" cell embodying the invention and cut away to show structure.

35 Fig. 5 is a sectional elevation of a "dry" cell embodying the anode of the invention.

40 In Figs. 2 and 3, like numerals designate like parts.

45 Referring more particularly to the drawing

there is shown in Figs. 2 and 3 a "wet" cell designed particularly for test purposes having case 1 containing an electrolyte 2. Submerged in the electrolyte 2 is the anode 3 which is held upon the insulating plate 4 by beeswax 5, which also covers the edge 6 of the anode so that only the face 7 is exposed to the electrolyte. The plate 4 may be formed of glass, synthetic resin or the like. It is convenient to make the anode face circular and 1 inch in diameter. A suitable insulated lead 8 is provided for making electrical connection to the anode. Spaced 0.6 inch away from the face 7 of the anode is the cathode plate 9. For the purpose of making efficiency tests, the cathode may have a rectangular shape 3 x 4 inches with the long dimension vertical as shown in Fig. 4. A suitable lead 10 is provided for making electrical connection with the cathode. For measuring the ampere hours output of the test cell an ammeter 11 connected in series with the variable resistance 12 may be used, as shown in Fig. 2.

Fig. 4 represents a preferred form of a "wet" cell assembled with the improved anode. As shown, the cell consists of a jar 13 of insulating material, such as glass or molded plastic, divided into an anode compartment 14 and a cathode compartment 15 by a partition 16. Partition 16 consists of a board or plate of insulating material such as glass or plastic, which is conveniently molded of phenol-formaldehyde resin. It is provided with a plurality of perforations 17 arranged in a regular pattern to permit the passage of electric current from one compartment to the other. On the cathode side of partition 16 is a porous filter medium 18 such as a sheet of filter paper, which serves as a liquid-permeable retainer for the contents of the cathode compartment 15. In compartment 14 is disposed the anode 19 consisting of a plate of the magnesium-mercury-alloy aforementioned, to which is secured a terminal rod 20, the plate 19 being immersed in a body of aqueous electrolyte 21. Cathode 22 in compartment 15 is a carbon rod having a terminal 23. The carbon rod 22 is embedded in a mass 24 of a depolarizer mix composed of manganese dioxide and finely divided carbon moistened with electrolyte.

In the "dry" cell shown in Fig. 5 the magnesium-mercury alloy anode constitutes the container 25. The cathode 26 is a carbon rod having a terminal cap 27 packed in a bobbin 28 of a depolarizer mass of manganese dioxide and carbon moistened with any suitable aqueous electrolyte such as one of those aforementioned. Between depolarizer 28 and the sides of the container is a body of gelled electrolyte 29. An insulating cup 30 of waxed paper, paper board or the like separates the depolarizer bobbin 28 from the bottom 31 of the container. A disc 32 of similar insulating material covers the top of the bobbin. A vent space 33 is provided above disc 32 which is closed by a vented insulating cover 34 of wax or resin.

The performance of the anode material of the invention is well illustrated by a series of tests employing a test cell having the form shown in Fig. 2, with the anode of Fig. 3, a cathode of carbon and having an electrolyte composed of an aqueous solution containing 150 grams of ammonium bromide and 5 grams of ammonium chromate per liter. The results of such tests are plotted in Fig. 1.

In each of the tests of the series using the form of cell of Fig. 2 a different anode was used, each being in the form of a circular piece of

rolled plate 1 inch in diameter. Each such anode differed one from the other as regards the mercury content which ranged in small increments from a blank with no mercury to 1.5 per cent by weight of mercury while iron content was about 0.002 per cent in each anode.

In obtaining the performance data with the cell of Fig. 2 each anode was weighed before assembling in the cell and the cell was discharged through the variable resistance 12 and ammeter 11 as shown in Fig. 2. During the discharge, the variable resistance 12 was constantly adjusted so as to maintain a substantially constant rate of discharge corresponding to a current density of 7 amperes per square foot of electrode (anode) surface exposed to the electrolyte. Each anode was allowed to discharge for 100 minutes. After discharging, each anode was removed from the cell cleaned and weighed. The difference in the weight of each anode before and after the test compared to the theoretical weight of metal corresponding to the number of coulombs of electricity produced was used in computing the efficiency according to the formula:

$$\text{per cent efficiency} = \frac{100 \times \text{coulombs obtained from cell}}{7940 \times \text{anode weight loss in grams}}$$

Efficiencies obtained by the foregoing tests were plotted as ordinates in Fig. 1 against the corresponding mercury content of the anode as abscissa. It will be observed that an unexpected increase in anode efficiency is realized when the mercury content of the anode is between about 0.16 and 0.7 per cent and that the maximum efficiency is obtained when the mercury content is about 0.5 per cent while the iron content is within the aforesaid range.

Further examples of "wet" cells of the form of Fig. 2, are tabulated in Tables I and II using an anode formed of the alloy composed of 0.5 per cent of mercury 0.002 per cent of iron, the balance being magnesium having a purity of 99.98 per cent.

Table I

| Cell Designation | Electrolyte Composition Concentration of Salts in Water                                                         | Per Cent Anode Efficiency <sup>1</sup> |
|------------------|-----------------------------------------------------------------------------------------------------------------|----------------------------------------|
| 1                | 150 g. p. L. NH <sub>4</sub> Br+Saturated with K <sub>2</sub> Cr <sub>2</sub> O <sub>7</sub> .                  | 80                                     |
| 2                | 150 g. p. L. NH <sub>4</sub> Br+Saturated with (NH <sub>4</sub> ) <sub>2</sub> Cr <sub>2</sub> O <sub>7</sub> . | 78                                     |
| 3                | 150 g. p. L. NH <sub>4</sub> Br+Saturated with (NH <sub>4</sub> ) <sub>2</sub> CrO <sub>4</sub> .               | 61                                     |
| 4                | 150 g. p. L. NH <sub>4</sub> Br+5 g. p. L. (NH <sub>4</sub> ) <sub>2</sub> CrO <sub>4</sub> .                   | 83                                     |

<sup>1</sup> With carbon plate cathode.

Referring to Table I, the "anode" efficiency was determined and computed in the manner already described.

Table II

| Cell Designation | Electrolyte Composition Concentration of Salts in Water                                                         | Initial Closed Circuit Voltage <sup>1</sup> |
|------------------|-----------------------------------------------------------------------------------------------------------------|---------------------------------------------|
| 1                | 150 g. p. L. NH <sub>4</sub> Cl+5 g. p. L. (NH <sub>4</sub> ) <sub>2</sub> CrO <sub>4</sub> .                   | 0.84                                        |
| 2                | 150 g. p. L. NH <sub>4</sub> Br+29 g. p. L. (NH <sub>4</sub> ) <sub>2</sub> CrO <sub>4</sub> .                  | 0.80                                        |
| 3                | 300 g. p. L. SrBr <sub>2</sub> ·6H <sub>2</sub> O+2 g. p. L. (NH <sub>4</sub> ) <sub>2</sub> CrO <sub>4</sub> . | 0.54                                        |

<sup>1</sup> Using platinized platinum cathode connected through 5 ohm resistor to anode.

As illustrative of "dry" cells, those tabulated in Table III are examples made up in D size in

the form shown in Fig. 5. In each cell the anode (cup 25) was composed of the alloy consisting of about 0.5 per cent of mercury and 0.001 per cent of iron, the balance being magnesium having a purity of 99.98 per cent. The cathode was a carbon rod imbedded in the depolarizer mix of 90 parts of manganese dioxide and 10 parts of acetylene black.

Table III

| Cell Designation | Electrolyte Composition Concentration of Salts in Water                                                 | Initial Cell Voltage | Discharge Tests                 |
|------------------|---------------------------------------------------------------------------------------------------------|----------------------|---------------------------------|
| 1.....           | 150 g. p. L. $\text{NH}_4\text{Br}$ + 50 g. p. L. $(\text{NH}_4)_2\text{CrO}_4$ .                       | 1.84                 | BA-30 <sup>1</sup><br>5.9 days. |
| 2.....           | 1000 g. p. L. $\text{SrBr}_2 \cdot 6\text{H}_2\text{O}$ + 0.05 g. p. L. $(\text{NH}_4)_2\text{CrO}_4$ . | 2.03                 | 11.2 days.                      |
| 3.....           | 1000 g. p. L. $\text{SrBr}_2 \cdot 6\text{H}_2\text{O}$ + 0.05 g. p. L. $(\text{NH}_4)_2\text{CrO}_4$ . | 2.03                 | BA-8 <sup>2</sup><br>138 hours. |

<sup>1</sup> Cell discharged for 4 minutes through a 6 $\frac{1}{2}$  ohm resistor twice each hour for 10 consecutive hours of each day 5 days a week until the cell voltage declines to 0.935. Total number of elapsed days from beginning to end of discharge test is recorded.

<sup>2</sup> Cell continuously discharged through a resistor of 83 $\frac{1}{2}$  ohms until cell voltage declined to 1.13 volts. The total number of hours of such discharge is recorded.

We claim:

1. In a primary cell having in combination an

aqueous electrolyte, an anode, and a cathode, the improvement which consists in forming the anode of magnesium alloyed with from 0.16 to 0.7 per cent by weight of mercury, the iron content of the alloy not exceeding 0.007 per cent.

5 2. In a primary cell having in combination an aqueous electrolyte, an anode, and a cathode, the improvement which consists in forming the anode of magnesium alloyed with about 0.5 per cent by weight of mercury, the iron content of the alloy not exceeding 0.007 per cent.

PERCY F. GEORGE.  
ASHFORD B. FRY.  
ROY C. KIRK.

## REFERENCES CITED

The following references are of record in the file of this patent:

## UNITED STATES PATENTS

| Number    | Name    | Date          |
|-----------|---------|---------------|
| 1,771,190 | Polcich | July 22, 1930 |
| 2,445,306 | Lawson  | July 13, 1948 |

## OTHER REFERENCES

Robinson, H. A., Trans. Electrochemical Socy., vol. 90 (1946), pages 499, 500.